

Nov. 6, 1928.

1,691,005

E. BURKE

FIBER INSULATOR AND METHOD OF MAKING THE SAME

Filed Sept. 11, 1925

*Fig.1*



*Fig.2*



*Fig.3*



*Fig.4*



*Fig.5*



*Fig.6*



*Fig.7*



*Fig.8*



*Inventor*  
*Edmund Burke*

*His Spc Jr.*

*By Attorney*

Patented Nov. 6, 1928.

1,691,005

# UNITED STATES PATENT OFFICE.

EDMUND BURKE, OF PORTLAND, MAINE, ASSIGNOR TO BROWN COMPANY, OF PORTLAND, MAINE, A CORPORATION OF MAINE.

## FIBER INSULATOR AND METHOD OF MAKING THE SAME.

Application filed September 11, 1925. Serial No. 55,851.

In the production of electric insulators various efforts have been made to utilize some substitute for porcelain or vitreous materials on account of their high cost and extreme fragility. The expense of such insulators and the difficulties involved in their shipment and handling has made the cost of initial installation a very heavy burden and the necessity for frequent replacement involves correspondingly heavy upkeep expense which is burdensome even to the large power companies.

A great variety of insulating substitutes have been devised and tried, but to the best of my knowledge have either not been successful or have not compared sufficiently favorable with the higher priced porcelain to warrant any considerable use. As I understand it, the porcelain insulator remains today the standard article for high tension lines at least in spite of all the expense and difficulty involved.

One of the difficulties involved in the production of fiber compound insulators seems to me to have arisen from a lack of understanding of the peculiar qualities of fiber. Vegetable fiber, especially the fiber of woody growths, such as are used in wood pulp, respond in marked degree to methods of handling. This has been recognized in paper making but has not apparently been recognized in the formation of such moulded articles as insulators. I have been able by a methodical application of some old and some new principles to form insulators of fiber compounds of high dielectric quality and at the same time of a tensile strength sufficient to make possible certain mechanical features which make these insulators available for general use, and which compare favorably with the very expensive porcelain insulators heretofore depended on.

In disclosing my invention I will take the production of an insulator of standard type, it being understood that such is merely illustrative and almost any type of insulator can be manufactured by my method by an observance of the principles disclosed herein by those skilled in the art. To show the steps involved, I have illustrated in the accompanying drawings the various steps in the formation of such an insulator and to these drawings I make reference by the usual characters. In the drawings:

Fig. 1 indicates the formation of a body of stock upon a mandrel.

Fig. 2 a section of such stock flattened out.

Fig. 3 another method of forming the body of stock.

Fig. 4 a section of such a body removed. 60

Fig. 5 is a sectional view of such a body subject to a preliminary forging.

Fig. 6 a similar view indicating the same impregnated.

Fig. 7 a similar view showing the insulator 65 finally forged, and

Fig. 8 a partly sectioned view showing the finished insulator.

In the preparation of stock for my insulator, I may take the usual or a slightly modified stock from the wet machine, forming it so as to wet lay the fibers loosely in a felting relation, with a considerable excess of water. This matter of excess of water is encouraged rather than discouraged in so many methods 70 of preparing stock. 75

This step may be accomplished by building up a body of the fiber by rolling it in a continuous film on the mandrel, as indicated in Fig. 1, or the fiber may be deposited as indicated in Fig. 3, by sluicing it wet into a cage which may advantageously be roughly shaped to give the general configuration of the article desired. 80

For example, I have endeavored to illustrate in Fig. 4 a mass of fiber F which has been roughly formed by sluicing into a cage C through which the excess water has filtered so that the fibers have settled together either without pressure or with a very slight or gentle pressure, just sufficient to bring the fiber mass to such a consistency that it can be handled. 85 90

This fiber mass should then, if necessary, be somewhat further dried. When it has 95 reached the state where the excess of water has been eliminated, it is first rough forged as indicated in Fig. 5, to form a groove member I. This shaping while still moist can be accomplished without any real disturbance of the fibers and it further brings the article to a more compacted state. The blanks may now be thoroughly dried and then impregnated in a vacuum tank with a suitable plastic which is preferably in part at least of 100 asphaltic nature. In practice I prefer to use a mixture of approximately one-half gilsonite and one-half pitch. 105

The result, as I have attempted to illustrate in Fig. 6, is an impregnated rough formed blank which is thoroughly impregnated and from which the water has been entirely removed.

The article in this condition I have indicated at I<sup>1</sup>. It is taken while still hot and subjected to a die forging under a considerable pressure. This produces an article as 10 indicated at I<sup>2</sup>, Fig. 7, which is formed true to the shape desired. In the form shown, it is provided with an axial boss i on its upper portion and a recess i<sup>2</sup> on its lower portion. It may be formed with any number of ribs as 15 at i<sup>3</sup> according to the type desired.

Such an article when cooled and allowed to harden provides an insulating unit which is capable of being worked to give it mechanical bondings such as the threadings S indicated 20 in Fig. 8. These threadings may be milled or otherwise cut in the insulator and will be found to have ample strength for any connection desired, whether they be metallic trimmings or whether they be inter-unit 25 bondings. Such cut surfaces are capable of a very strong cement, as by the impregnating compound itself, or by other cementitious material, and where such threaded parts on the insulator units are brought together as in 30 multiple petticoat types and so cemented, the insulator becomes practically a unitary article substantially homogeneous throughout.

In practice the impregnation is carried on for two to three days to secure a very complete permeation and a very complete extraction of the water. The impregnating compound may be proportioned so as to have any desired melting point in the usual manner known to those skilled in the art. Insulators 35 so prepared have a very high electric resistance and may be formed in the most approved pattern and design. Furthermore, they are capable of multiple assembly so as to make 40 possible an insulator of any desired resistance which can be built up even on the job and

which when built up is a strong and serviceable article which will not only withstand the incidents of ordinary line service, but which will even withstand such abuse as sniping or other attempts at breakage.

Insulators so formed and of such strength 50 may be shipped and handled with the greatest freedom in sharp contra-distinction to the expensive barrel packing necessary for porcelain insulators which in many cases have to be 55 packed one to a barrel for safety.

As I have stated above, the type of insulator shown is purely illustrative. It will be further understood that the method outlined is selected for characteristic simplicity. It 60 may be varied as to various steps. The fibers may be cooled or laid in any desired manner and the article produced by any known steps consistent with the ultimate form desired and the maintenance of the character of the fiber, 65 all without departing from the spirit of my invention.

What I therefore claim and desire to secure by Letters Patent is:

1. The method of making petticoat insulators which consists in preparing a blank of wet laid fibrous stock, in rough shaping said blank while moist, in drying the rough shaped blank, in impregnating the blank with a dielectric thermo-plastic and die finishing 75 under pressure.

2. The method of making petticoat insulators which consists in preparing a blank of wet laid fibrous stock, in rough shaping said blank while moist, in drying the rough shaped 80 blank, in impregnating the blank with a dielectric thermo-plastic and die finishing under pressure and in tool fitting for assembly.

3. A compressed fiber insulator of wet 85 laid fibrous stock having a transverse fiber trend and impregnated with a dielectric thermo-plastic.

In testimony whereof I affix my signature.  
EDMUND BURKE.